

# UNITED STATES PATENT OFFICE.

GILBERT RIGG, OF PALMERTON, PENNSYLVANIA, ASSIGNOR TO NEW JERSEY ZINC COMPANY, OF NEW YORK, N. Y., A CORPORATION OF NEW JERSEY.

## EXPLOSIVE SHELL.

1,235,245.

Specification of Letters Patent. Patented July 31, 1917.

No Drawing.

Application filed February 8, 1916. Serial No. 76,022.

*To all whom it may concern:*

Be it known that I, GILBERT Rigg, a citizen of the United States, residing at Palmerton, Carbon county, State of Pennsylvania, have invented certain new and useful Improvements in Explosive Shells; and I do hereby declare the following to be a full, clear, and exact description of the invention, such as will enable others skilled 10 in the art to which it appertains to make and use the same.

This invention relates to explosive shells, and to smoke-producing compositions for use therein.

15 I have found that the blue powder, which is obtained in the smelting of zinc, is a valuable substitute for magnesium as a smoke-producing constituent of explosive shells and compositions therefor. The blue powder 20 appears to particular advantage when it is intimately combined with other constituents, notably black gun powder, which will exert a stimulating action upon the conversion of the blue powder into a visible "smoke".

25 As is well understood in the art, it is desirable that a smoke-producing composition for explosive shells should give a dense smoke which will have a reasonable capacity for hanging, thereby indicating the position 30 of explosion of the shell with sufficient accuracy and for a suitable time to permit observation. I have found that compositions containing the blue powder, and in particular compositions containing the blue powder 35 with black gun powder, are well adapted for this purpose.

The blue powder used according to the present invention is the blue powder obtained in the distillation of zinc, being that 40 part of the distillate partially oxidized, so that it is made up of fine particles of zinc coated with zinc oxid. In the action of this fine blue powder, the intimate mixture of the metallic zinc and zinc oxid, when incorporated in a smoke-producing composition 45 with black gun powder, appears to have a favorable influence upon the smoke-producing qualities of the composition.

By varying the proportions of the black gun 50 powder, the composition can be made either of good or weak explosive properties, or even without explosive properties. I have obtained good results with from 30% to 60% of the blue powder mixed with from 55 70% to 40% of gun powder. I have even

obtained a good explosion and a white smoke by the use of a composition made up of 10% of the blue powder and 90% of the gun powder. With equal parts of the gun powder and blue powder a weak explosion 60 was obtained, with a good smoke production. Practically no explosion was obtained with a mixture of 30% gun powder and 70% blue powder, while the smoke was nevertheless of a dense nature. A dense smoke is also 65 produced by a mixture of about 25% gun powder and 75% blue powder. With this proportion, however, as well as with compositions containing equal parts of the blue powder and gun powder, or mixtures richer 70 than 50% in blue powder, the production of the smoke is somewhat slower, so that the smoke is produced in a somewhat progressive manner instead of instantaneously. This smoke production is, however, desirable 75 in some instances, delaying or continuing the smoke production so that it can be more readily observed.

As compared with smoke-producing mixtures containing magnesium, which unite 80 readily and with explosive violence, the compositions containing blue powder ignite less rapidly and with less violence. In smoke production, however, the blue powder forms an important substitute for magnesium, with 85 advantages not possessed by the magnesium compositions.

As above noted, gun powder appears of particular advantage as a constituent of smoke-producing compositions with the blue 90 powder, coöperating with it in the production of the desired "smoke" from the zinc and zinc oxid of the blue powder.

In utilizing the novel smoke-producing composition of the present invention in the 95 manufacture of explosive shells, the usual methods of incorporation are available, the shell containing the composition having like advantages to those above indicated.

I claim:-

1. An explosive shell comprising a smoke-producing composition containing blue powder and black gun powder; substantially as described.
2. An explosive shell containing a smoke 105 producing composition of blue powder and black gun-powder in suitable proportions to form a slow burning composition, substantially as described.
3. An explosive shell containing a smoke 110

producing composition of blue powder and black gun-powder in the proportions of from thirty to sixty per cent. of the blue powder and of from forty to seventy per 5 cent. of the black gun-powder, substantially as described.

4. An explosive composition comprising blue powder and black gun powder; substantially as described.

16 5. An explosive composition comprising

blue powder and black gun powder in suitable proportions to form a slow burning composition; substantially as described.

6. An explosive composition comprising blue powder and black gun-powder in the 15 proportions of from thirty to sixty per cent. of the blue powder and of from forty to seventy per cent. of the gun-powder.

In testimony whereof I affix my signature.

GILBERT RIGG